

## UNITED STATES PATENT OFFICE

2,196,963

## STABILIZED MINERAL OIL COMPOSITION

Everett W. Fuller, Woodbury, N. J., assignor to  
Socony-Vacuum Oil Company, Incorporated,  
New York, N. Y., a corporation of New York

No Drawing. Application February 1, 1939,  
Serial No. 253,990

9 Claims. (Cl. 87—9)

This invention is concerned with the stabilization of viscous mineral oil fractions against the harmful effects of oxidation or deterioration with use through the use of so-called "anti-oxidants" or "oxidation-inhibitors." The invention is more specifically related to the improvement or stabilization of such mineral oil fractions by the use of novel compounds, or a novel class of compounds, which when admixed with a viscous mineral oil in minor proportions will prevent or delay undesirable changes taking place in the oil.

As is well known to those familiar with the art, substantially all the various fractions obtained from mineral oils and refined for their various uses are susceptible to oxidation. The susceptibility of an oil fraction to oxidation and the manner in which oxidation manifests itself within the oil varies with the type and degree of refinement to which the oil has been subjected and with the conditions under which it is used or tested. In other words, the products formed in an oil fraction as a result of oxidation and the degree to which they are formed depends upon the extent to which the various unstable constituents or constituents which may act as oxidation catalysts have been removed by refining operations, and also upon the conditions of use.

A highly refined viscous oil, for example, which is one that has been refined by treatment with fuming sulfuric acid or other means or combinations such as  $\text{AlCl}_3$ , solvents and acids (or with large quantities of concentrated sulfuric acid), tends to form relatively large amounts of acidic constituents when subjected to oxidizing conditions. The presence of catalytic materials such as copper does not appear to affect appreciably the oxidation of highly refined oils, and such oils are less prone to the formation of colored bodies or of insoluble sludge. The formation of acidic bodies, however, is highly undesirable for most applications of these oils. For example, when used as an insulating or cooling oil in electrical equipment such as transformers or capacitors an increase in acidic bodies tends to lower the dielectric strength of the oil and has other harmful effects which are undesirable. The acids are corrosive to metals and thus reduce the useful life of the oils as lubricants or for other purposes in which they come in contact with metals, and the acidic materials are also injurious in textile lubricants and in spray oils.

Moderately refined oils, that is, oils that have been refined by treatment with only moderate amounts of sulfuric acid, or other refining agents, tend to form relatively small amounts of acidic

oxidation products as compared with highly refined oils, but they undergo material color depreciation and form considerable amounts of sludge. The changes taking place in these oils are appreciably accelerated by the presence of metal catalysts such as copper. Sufficient acid is generally formed to cause some reduction in the dielectric strength of these oils, but the principal objection to them is their tendency to deposit sludge which interferes with heat transfer in transformers and turbines and also causes plugging of oil feed lines in lubricating systems.

Solvent-refined oils in general, which have been prepared by treatment with selective solvents, such as chlorex, phenol, furfural, etc., resemble the moderately refined acid-treated oils in that their oxidation is accelerated by the presence of metals such as copper and further in that it is attended by substantial color depreciation and sludge formation. Acid formation is usually greater than in the case of moderately acid-refined oils, but considerably less than with highly refined oils. Both sludge and acid formation lower their value for many purposes, such as electrical insulation, lubrication, etc. Also, solvent-refined oils have found extensive use as lubricants for internal combustion engines because of their high viscosity index, but under the conditions of use encountered in crankcases such oils develop constituents which are corrosive toward certain metal bearings such as the cadmium-silver bearings, etc., which are sometimes used.

It is to be understood that this classification of oils as "highly refined," "moderately refined" and "solvent refined" is by no means limiting and that there can exist oils whose refining and blending has been such as to make them intermediate in properties between the types set up. Thus, response to inhibitors may be said to depend entirely upon the type of oxidation and end products of oxidation of an oil, which in turn depends largely upon the degree of refining this oil has had. Further the degree of refining required to produce these types of oils varies with the crude source so that any one refining procedure may produce either a highly refined oil or a moderately refined oil, depending upon the crude source. Pennsylvania type oils, for example, require much less refining to produce highly refined oils than the Coastal type of oils.

The use of oxidation inhibitors for the purpose of stabilizing a viscous mineral oil fraction against the deleterious effects of oxidation discussed above is well known. Since the action of

these inhibiting materials is apparently catalytic, the problem of their development is a difficult one and is evidently influenced to a large degree by the oxidizable constituents which are in the oil following a particular refining treatment. Thus a particular inhibitor or class of inhibitors may be effective to stabilize a highly refined oil against acid formation while the same inhibitor may have no appreciable effect upon acid, color or sludge formation in a moderately refined oil and vice versa. This same inhibitor may or may not be effective in inhibiting acid, sludge and color formation in a solvent-refined oil and may or may not be effective to inhibit the corrosive action of a solvent-refined oil toward metals such, for example, as the various normally corroded alloys typified by cadmium-silver bearings.

The present invention is particularly concerned with a class of compounds which have been found to be highly effective as inhibitors of acid formation in highly refined oils. It is also concerned with the stabilization of moderately refined oils and the inhibition of alloy corrosion with solvent-refined oils, but in these latter two instances one specific compound of the class appears to exhibit outstanding superiority over the other tested member of the general group or class contemplated herein.

The invention is predicated upon the discovery that certain of the thio-aldehydes are highly effective in small amounts as inhibitors of acid formation in highly refined oils. Two specific compounds in the class, namely trithioformaldehyde and trithioacetaldehyde, were tested in this regard and both were shown to be highly effective. In the moderately refined oil and the solvent-refined oil, however, the trithioformaldehyde was not found to be of particular effectiveness. This compound is only slightly soluble in mineral oil, however, and it is likely that this may have been the major factor contributing to the relatively poor showing which it made on these particular oil fractions. In this regard it will be understood that my invention contemplates the use of a suitable solvent such as benzol or a solubilizing alcohol to facilitate admixture of the inhibiting agent with the oil.

The thioaldehydes, contemplated herein as anti-oxidants for viscous mineral oils, are best known in their tripolymeric form, such polymers being illustrated by trithioformaldehyde ( $\text{CH}_3\text{S}$ )<sub>3</sub> and trithioacetaldehyde ( $\text{CH}_3\text{CHS}$ )<sub>3</sub>. They may be prepared by reacting the corresponding aldehyde with hydrogen sulfide and hydrochloric acid (Baumann, Berichte 23, 60). Other methods may also be used such as treating an aldehyde with sodium thiosulfate in the presence of ICI (Schmidt, Berichte 40, 365).

The following examples illustrate the effectiveness of the class of compounds and certain specific members within the class contemplated herein as anti-oxidants for mineral oil fractions.

#### EXAMPLE I

##### Highly refined oils

The oil employed in this test was of the "highly refined" type used in transformers and the like which had been obtained from a Coastal distillate by successive treatments with 98 per cent sulfuric acid in the ratio of 40 lbs. per bbl. and 103 per cent oleum in the ratio of 180 lbs. per bbl. followed by neutralization, washing, and clay percolation. The refined oil had a specific gravity of 0.871, a flash point of 310° F. and a

Saybolt Universal viscosity of 69 seconds at 100° F.

The test used, known as the modified German tar test, involved heating a 150 gram sample of the oil at a temperature of 120° C. while bubbling oxygen gas through the oil for a period of 70 hours. The amount of acidic oxidation products thus formed was found (a) by extracting the oil with alcoholic soda, neutralizing the extract and then weighing the precipitated material, which is calculated as per cent acidic tar, and (b) by titrating the acids formed in the oil with alcoholic KOH and expressing the result as the neutralization number (N. N.) which is the milligrams of KOH required to neutralize the acid in one gram of oil. The results of this test are listed in Table I below where oils "A" and "A<sub>1</sub>" represent the oil alone, oil "B" indicates oil "A" with 0.05 per cent trithioformaldehyde and oil "C" indicates oil "A<sub>1</sub>" with 0.10 per cent tri-thioacetaldehyde.

Table I

| Oil            | Acidic products formed |
|----------------|------------------------|
| A              | 15% acidic tar.        |
| B              | 0.02% acidic tar.      |
| A <sub>1</sub> | 25.0 N. N.             |
| C              | 0.02 N. N.             |

From the foregoing results it will be seen that both of the thioaldehydes tested are very effective in minute quantities as inhibitors of acid formation in highly refined oils.

#### EXAMPLE II

##### Moderately refined oil

The oil used in this test was a "moderately refined" light turbine oil stock obtained from a blend of 92 per cent Mid-Continent distillate and 8 per cent Coastal distillate by treatment with 70 lbs. of 98 per cent sulfuric acid per bbl., followed by neutralization, washing and clay percolation. The refined oil had a specific gravity of 0.879, a flash point of 385° F. and S. U. viscosity of 152 seconds at 100° F.

In testing moderately refined oils of the turbine oil type for deterioration under the influence of oxidation the so-called "Brown-Boveri turbine oil test" was used. In this test a sample of oil is heated to a temperature of 110° C. in air for 72 hours with a piece of copper foil in the oil, the results observed being final color, and acidity, expressed as neutralization number (N. N.).

This oil, blended with 0.10 per cent tri-thioacetaldehyde, when subjected to the foregoing test showed a Lovibond color of 8 and a neutralization number of 0.05 as compared with the oil alone, which after subjection to the same test had a Lovibond color of 15 and a neutralization number of 0.07. As has been pointed out above, the trithioformaldehyde, probably because of its low solubility, was not shown by this test to be an effective anti-oxidant for moderately refined oil, and the results obtained are not given since improved results may be obtainable through the use of a solvent.

#### EXAMPLE III

##### Solvent-refined oil

The two illustrative thioformaldehydes described herein were also tested for their effect upon the corrosive action of solvent-refined motor oils toward alloys such, for example, as cad-

mium-silver bearings of the type normally corroded by such oils under conditions of use. The oil used was an S. A. E. 20 motor oil obtained from a Pennsylvania mixed neutral residuum stock by solvent extraction with chlorex. It had a specific gravity of 0.872, a flash point of 435° F. and an S. U. viscosity of 318 seconds at 100° F.

The test used involved immersing a 6 gram section of a cadmium-silver automobile bearing in a 30 gram sample of oil, heating the oil to a temperature of 175° C. and bubbling air therethrough against the surface of the bearing for a period of 22 hours. The loss in weight of the bearing section is a measure of the corrosion which has taken place.

Here again the trithioformaldehyde, probably because of low solubility, did not show material effectiveness, but the trithioacetaldehyde when blended with this oil in the amount of 0.10 per cent reduced the loss in weight of the test specimen from 41 mg. (for the oil alone) to 1 mg. (for the blend containing trithioacetaldehyde).

It is to be understood that the terms "highly refined", "moderately refined" and "solvent-refined" as used herein have reference to oils corresponding substantially in their manner of deterioration and inhibitor response to the examples given and are not necessarily restricted to oils obtained by particular refining operations. As has been previously pointed out, the final characteristics in an oil fraction are effected by the crude from which the oil is obtained as well as the refining treatment and by selection of the crude stock an oil of the "highly refined" type may be obtained by a treatment which on another crude stock would yield an oil having the characteristics of a "moderately refined" oil.

The amount of the inhibitor used may be varied, depending upon the oil fraction, from about 0.05 per cent to about 2.0 per cent more or less, depending upon its solubility and whether an admixing solvent is employed. In general the amount satisfactory for substantial inhibition will be in the neighborhood of from about 0.05 per cent to about 0.1 per cent.

I claim:

1. A viscous mineral oil fraction having in admixture therewith a minor proportion of a thioaldehyde in an amount sufficient to inhibit the deleterious effects of oxidation on the oil.

2. An improved mineral oil composition comprising a highly refined viscous mineral oil fraction and in admixture therewith a minor proportion of a thioaldehyde in an amount sufficient to inhibit the deleterious effects of oxidation on the oil. 5

3. An improved mineral oil composition comprising a viscous mineral oil fraction and in admixture therewith a minor proportion of trithioacetaldehyde in an amount sufficient to inhibit the deleterious effects of oxidation on the oil. 10

4. An improved mineral oil composition comprising a highly refined viscous mineral oil fraction and in admixture therewith a minor proportion of a compound selected from the group consisting of trithioformaldehyde and trithioacetaldehyde, said compound being present in the oil in an amount sufficient to inhibit the deleterious effects of oxidation on the oil. 15

5. An improved mineral oil composition comprising a viscous mineral oil fraction having in 20 admixture therewith a minor proportion of trithioformaldehyde in an amount sufficient to inhibit the deleterious effects of oxidation on the oil.

6. An improved mineral oil composition comprising a viscous mineral oil fraction selected from the group consisting of highly refined oils, moderately refined oils and solvent-refined oils, and in admixture therewith a minor proportion of trithioacetaldehyde in an amount sufficient 30 to inhibit the deleterious effects of oxidation on the oil. 25

7. A viscous mineral oil fraction having in admixture therewith a thioaldehyde in an amount of from about 0.05 per cent to about 0.1 per cent 35 sufficient to inhibit the deleterious effects of oxidation on the oil.

8. An improved mineral oil composition comprising a viscous mineral oil fraction normally subject to deterioration under oxidizing conditions and in admixture therewith in minor proportion, sufficient to retard said deterioration, a compound selected from the group consisting of trithioformaldehyde and trithioacetaldehyde. 40

9. A viscous mineral oil fraction having in admixture therewith a minor proportion of an alkyl thioaldehyde in an amount sufficient to inhibit the deleterious effects of oxidation. 45

EVERETT W. FULLER. 50